

March 18, 1930.

J. E. HOY

1,751,038

CASTING MAGNESIUM AND ALLOYS THEREOF

Filed July 3, 1926



Fig. 1



Fig. 2



Fig. 3.

INVENTOR.

John E. Hoy

BY  
Fay Oberlin & Fay  
ATTORNEYS

## UNITED STATES PATENT OFFICE

JOHN E. HOY, OF MIDLAND, MICHIGAN, ASSIGNOR TO THE DOW CHEMICAL COMPANY,  
OF MIDLAND, MICHIGAN, A CORPORATION OF MICHIGAN

## CASTING MAGNESIUM AND ALLOYS THEREOF

Application filed July 3, 1926. Serial No. 120,426.

While the present improvements relate more particularly to the casting of magnesium and so-called light metal alloys in which magnesium is the predominant constituent, it will be understood that the improved method and apparatus involved are equally adaptable for the casting of any similar readily oxidizable metal. The difficulties encountered in melting and handling in 5 molten state magnesium or an alloy largely composed of this metal are well known and these difficulties are still present when it is attempted to introduce such metal into a mold in any process of casting. For example, when sand castings are made in the ordinary way by simply pouring the molten magnesium or light alloy metal in the sand mold, there is a very pronounced tendency for the metal to burn in the sprue. Even if the 10 burning is not serious enough to prevent the cast article from being properly finished when removed from the mold, a certain loss of metal, due to oxidation, is inevitable, and of course the cleaner the casting, the more easily 15 may the finishing operation be carried out.

It has heretofore been proposed to overcome these difficulties specifically in casting magnesium and alloys containing the same by dusting the mold prior to casting the metal 20 with sulphur or equivalent material capable of giving off in contact with the molten metal a vapor which is more easily oxidizable than magnesium. This procedure, however, has the objection that it is obviously difficult 25 correctly to gauge the amount of sulphur or equivalent material thus used, and particularly if an excess is applied to the surface either of the mold proper or the core, so much vapor may be generated that some of 30 it becomes entrapped during the period that the metal is solidifying, the result being blow-holes or surface shrinks in the casting. Furthermore, the sulphur or equivalent material has to be applied or dusted onto the mold so 35 that the method in question is obviously not

applicable where a metal mold is employed, because of the non-porous character of the latter.

The present improved method has as its object to generate directly in the mold cavity 50 a gas that is inert toward the metal being cast, and specifically sulphur dioxide, in an amount sufficient to displace the air normally filling such cavity but without danger of sulphur vapor becoming entrapped and generating an excessive amount of gas at some point. My improved method further permits of the 55 convenient regulation of the amount of sulphur dioxide for example, that is thus introduced into or supplying to the mold cavity. So that there will be no unnecessary wastage 60 on the one hand or insufficient amount of gas generated, on the other hand.

To the accomplishment of the foregoing 65 and related ends, the invention, then, consists of the steps hereinafter fully described and particularly pointed out in the claims, the annexed drawing and the following description setting forth in detail certain means and mode of carrying out the invention, such disclosed means and mode illustrating, however, but one of various ways in which the principle 70 of the invention may be used.

In said annexed drawing:—

Fig. 1 is a central vertical section thru a 75 mold constructed and arranged to carry out my improved method; Fig. 2 is a broken top plan view of the same; and Fig. 3 is a section taken on a plane indicated by line III—III, 80 Fig. 1.

The mold thus illustrated is specifically designed for casting a piston for an internal combustion engine or like hollow article of general cylindrical form. The mold part 1 85 will preferably be of metal, e. g. cast iron, as is commonly used in foundries at the present time for casting light metal pistons, but such mold may be made of sand if desired. Such permanent mold has a cavity 2 that conforms 90 with the exterior shape of the article to be

cast and an enlarged space 3 continuous with the upper end of such cavity whereby a lateral offset shoulder 4 is provided that encircles such cavity.

6 The core 6, which may be either of sand or of collapsible metal parts, is of course separable from the mold 1 and is formed with an enlargement 7 at its upper end adapted to fit the enlarged portion 3 of the mold cavity, the 10 shoulder 8 between such enlargement and the core proper resting on the offset 4 in the mold when the parts are assembled.

7 The enlargement 7 and such shoulder 8 of the core or else the complementary portions of the mold 1 are so formed as to leave 15 vent holes 9 thru which air or other gases may escape from the mold cavity, when the casting is poured. For the purpose of introducing the molten metal, the core is provided with a central sprue 11, the lower portion 20 of which communicates thru a gate 12 with the mold cavity in which the casting is to be formed.

8 A spoon-like container 13 preferably of 25 metal is provided so as to be adapted to receive and handle a quantity of burning sulphur, this container being supported by means of a handle extension 13<sup>a</sup> from the under side of a closure 14 removably fitted 30 to the upper end of the sprue level. A ring 15 or the like on said closure enables the latter to be lifted from or placing in the sprue opening as occasion may require.

9 In operation, after the mold part 1 has 35 been preliminarily warmed up as will be particularly desirable where such part is of metal, the core is placed in such mold in the conventional way. Thereupon, the spoon 12 is inserted into the sprue so as to occupy 40 a portion in the lower end thereof as illustrated in Fig. 1, such spoon having had previously placed therein a quantity of burning sulphur or of sulphur which is subsequently ignited before the spoon is thus introduced 45 into the sprue. Upon being left to stand for a few seconds, the sulphur will consume oxygen in the air confined in the mold cavity and at the same time more or less fill such cavity with sulphur dioxide, it being noted 50 that the sprue freely communicates with the main cavity thru the gate 12. When ready to pour the metal, the spoon is removed and the heavy gas generated by the combustion of the sulphur in the sprue is expelled forcibly 55 into the mold cavity, finally escaping thru the vents 9, which as explained above are so constructed as to pass around the core, and which are of suitable size that molten metal will solidify or freeze therein instead 60 of passing entirely thru.

65 As an example of a material that will generate a suitable inert gas, para dichlor-benzol may be named, altho this material has the disadvantage that the gases generated are more obnoxious than the sulphur dioxide

70 formed by burning sulphur, as also naphthalene, carbon tetrachloride and fuel oil. In no case, however, does the material used thus to generate the gas in question come into direct contact with the surfaces of the mold parts that define the casting. There is, accordingly no danger of an excessive amount of such gas being generated with resultant formation of blow-holes or surface shrinks.

75 Other modes of applying the principle of my invention may be employed instead of the one explained, change being made as regards the apparatus and the process or method herein disclosed, provided the means or steps stated by any of the following claims 80 or the equivalent of such stated means or steps be employed.

I therefore particularly point out and distinctly claim as my invention:—

85 1. A method of casting a readily oxidizable metal or an alloy containing the same, which comprises eliminating oxygen from the path of the molten metal on its way to and within the mold cavity by igniting an oxygen-consuming material in the path of the metal and out of contact with the mold surface.

90 2. A method of casting a readily oxidizable metal or an alloy containing the same, which comprises eliminating oxygen from the path of the molten metal on its way to and within the mold cavity by igniting a sulphur-containing material in the path of the metal and out of contact with the mold surface.

95 3. In a method of casting a readily oxidizable metal or an alloy containing the same, the steps which consist in eliminating air from the mold cavity and the pouring inlet thereto as well, by supporting in the inlet a quantity of material capable of generating a gas inert toward the metal being cast, and treating such material to generate such gas.

100 4. In a method of casting a readily oxidizable metal or an alloy containing the same, the steps which consist in eliminating air from the mold cavity and the pouring inlet thereto as well, by supporting in the inlet a quantity of sulphur, and igniting such sulphur, whereby the mold cavity is substantially filled with sulphur vapor and sulphur dioxide.

105 5. In apparatus for casting a readily oxidizable metal or alloy thereof, the combination with a mold including a core formed with a sprue having a gate to the mold cavity proper, of a container for gas-generating material arranged and constructed to be supported in such sprue.

110 6. In apparatus for casting a readily oxidizable metal or alloy thereof, the combination with a mold including a core formed with a sprue having a gate to the mold cavity proper, of a removable closure for the upper end of said sprue, and a container for a gas-

130

75

80

85

90

95

100

105

110

115

120

125

130

generating material supported from said closure.

7. In apparatus for casting a readily oxidizable metal or alloy thereof, the combination with a mold including a core formed with a sprue having a gate to the mold cavity proper, of a removable closure for the upper end of said sprue, and a container adapted to receive and hold a quantity of burning sulphur supported from said closure.

10 Signed by me this 22nd day of June, 1926.  
JOHN E. HOY.

15

20

25

30

35

40

45

50

55

60

65